

# United States Patent Office

2,860,971

Patented Nov. 18, 1958

1

2,860,971

## TITANIUM BASE ALLOYS

Harold Margolin, Mount Vernon, and William Frank Kirk, Bronx, N. Y., assignors to Kennecott Copper Corporation, New York, N. Y., a corporation of New York

No Drawing. Application October 16, 1956  
Serial No. 616,120

7 Claims. (Cl. 75—175.5)

This invention relates to titanium base alloys, and provides improved titanium base alloys comprising lead, aluminum, vanadium and tin with or without zirconium, as the essential alloying metals. The alloys of this invention comprise up to about 4% lead, up to about 7% aluminum, up to about 2.5% vanadium, up to about 20 2.5% tin, and when zirconium is included it is used in

2

good ductility and other desirable properties including good machinability, high modulus of elasticity, good cold workability and good elevated temperature properties.

The improved titanium base alloys of the invention accordingly comprise titanium as the major constituent, and from 0.1% to 4% of lead, from 3% to 7% of aluminum, from 0.5% to 2.8% of vanadium, from 0.5% to 2.5% of tin, and up to 4%, preferably from 0.5% to 3.5% of zirconium, when this metal is used. Oxygen 10 and nitrogen are considered to be objectionable impurities in these alloys and, if present should, in the aggregate, be in an amount less than about 0.2%. It is to be understood that the alloys may include the usual impurities contained in the ordinary commercial metals used in forming the alloys, and small amounts of one or more other metals which do not alter in any practical sense the characteristics of the alloys.

Typical titanium base alloys of this invention are illustrated in the following Table I which shows their compositions and mechanical properties. The titanium is the unrecorded balance.

Table I

| Alloy No. | Analyzed Composition |            |           |            |            | Specific Gravity | Tensile Strength (p. s. i.) | 0.2% Off. Y. S. (p. s. i.) | Percent Elong. (1") | Percent Red. in Area | Modulus of Elasticity (p. s. i. $\times 10^{-6}$ ) | VHN (10 kg.) | Treatment* |
|-----------|----------------------|------------|-----------|------------|------------|------------------|-----------------------------|----------------------------|---------------------|----------------------|----------------------------------------------------|--------------|------------|
|           | Percent Pb           | Percent Al | Percent V | Percent Sn | Percent Zr |                  |                             |                            |                     |                      |                                                    |              |            |
| 1.....    | 1.38                 | 3.29       | 2.13      | 2.28       |            | 4.59             | 146,800                     | 130,000                    | 11.5                | 36.0                 | 17.1                                               | 327          | F          |
| 2.....    | 0.74                 | 5.30       | 1.17      | 1.10       |            | 4.51             | 140,000                     | 135,400                    | 13.5                | 38.6                 | 19.1                                               | 327          | A          |
| 3.....    | 0.87                 | 5.27       | 2.11      | 2.09       |            | 4.54             | 140,000                     | 136,000                    | 12.8                | 37.7                 | 18.6                                               | 367          | B          |
| 4.....    | 1.36                 | 5.30       | 1.02      | 1.18       |            | 4.52             | 140,300                     | 134,200                    | 13.6                | 37.8                 | 18.3                                               | 336          | C          |
| 5.....    | 1.22                 | 5.46       | 2.13      | 2.23       |            | 4.52             | 140,000                     | 134,200                    | 12.5                | 40.7                 | 18.2                                               | 339          | A          |
| 6.....    | 0.09                 | 5.89       | 2.55      | 2.34       |            | 4.48             | 142,000                     | 140,000                    | 10.8                | 40.2                 | 18.9                                               | 327          | D          |
| 7.....    | 2.02                 | 5.85       | 2.69      | 2.54       |            | 4.55             | 147,000                     | 141,500                    | 13.4                | 45.2                 | 18.7                                               | 339          | D          |
| 8.....    | 1.96                 | 5.69       | 0.68      | 0.53       |            | 4.46             | 147,600                     | 141,400                    | 12.1                | 25.1                 | 19.9                                               | 333          | G          |
| 9.....    | 0.78                 | 6.36       | 1.04      | 1.17       |            | 4.48             | 152,000                     | 150,000                    | 14.0                | 39.3                 | 18.9                                               | 348          | A          |
| 10.....   | 0.96                 | 6.78       | 2.18      | 2.07       |            | 4.52             | 152,000                     | 149,500                    | 13.3                | 33.8                 | 18.9                                               | 363          | B          |
| 11.....   | 0.17                 | 7.45       | 0.72      | 0.87       |            | 4.41             | 153,300                     | 150,000                    | 12.0                | 27.9                 | 18.8                                               | 360          | H          |
| 12.....   | 0.86                 | 5.22       | 1.09      | 2.27       | 3.06       | 4.56             | 161,500                     | 160,200                    | 9.7                 | 19.6                 | 17.6                                               | 354          | C          |

\*A—As forged and heated for 24 hrs. at 500° C. and water quenched.

\*B—As forged and heated for 24 hrs. at 400° C. and water quenched.

\*C—As forged and heated for 2 hrs. at 775° C. and water quenched and heated for 24 hrs. at 500° C. and again water quenched.

\*D—As forged.

\*E—As forged and heated for 34 hr. at 1050° C. and water quenched.

\*F—As forged and heated for 1 hr. at 900° C. and water quenched.

\*G—As forged and heated for 1 hr. at 900° C. and water quenched and heated for 24 hrs. at 500° C. and again water quenched.

\*H—As forged and heated for 2 hrs. at 775° C. and air cooled.

\*I—As forged and heated for 2 hrs. at 775° C. and water quenched.

amounts up to about 4%. The alloys of the invention are characterized by very good tensile strength, high ratio of yield strength to tensile strength combined with

The alloys of this invention have very good elevated temperature properties which are shown in Table II for the temperature of 1020° F.

Table II

[Elevated temperature properties at 550° C. All specimens prevailing heat-treated 500° C. for 24 hours.]

| Alloy No. | Analyzed Composition |            |           |            | Specific Gravity | Tensile Strength (p. s. i.) | 0.2% Off. Yield Str. (p. s. i.) | Percent Elonga-tion (1") | Percent Red. in Area |
|-----------|----------------------|------------|-----------|------------|------------------|-----------------------------|---------------------------------|--------------------------|----------------------|
|           | Percent Pb           | Percent Al | Percent V | Percent Sn |                  |                             |                                 |                          |                      |
| 13.....   | 0.90                 | 3.05       | 2.03      | 2.15       | 4.56             | 68,900                      | 64,200                          | 14.4                     | 65.5                 |
| 1.....    | 1.38                 | 3.29       | 2.13      | 2.28       | 4.59             | 83,600                      | 78,400                          | 13.4                     | 65.1                 |
| 2.....    | 0.74                 | 5.30       | 1.17      | 1.10       | 4.51             | 91,200                      | 83,600                          | 11.4                     | 46.0                 |
| 3.....    | 0.87                 | 5.27       | 2.11      | 2.09       | 4.54             | 97,100                      | 92,100                          | 8.1                      | 33.6                 |
| 9.....    | 0.78                 | 6.37       | 1.04      | 1.17       | 4.48             | 97,300                      | 84,400                          | 11.9                     | 39.8                 |
| 10.....   | 0.96                 | 6.78       | 2.18      | 2.07       | 4.52             | 105,800                     | -----                           | 7.0                      | 30.5                 |

We claim:

1. Titanium base alloys consisting essentially of from 0.1% to 4% of lead, from 3% to 7% of aluminum, from 0.5% to 2.8% of vanadium, from 0.5% to 2.5% of tin and the balance of alloying metal being titanium, 20 said alloys having tensile strengths in excess of 136,000 p. s. i. coupled with good ductility, as represented by a reduction in area of at least 8.7%.

2. Titanium base alloys consisting essentially of from 0.1% to 2.5% of lead, from 3% to 7% of aluminum, 25 from 0.5% to 2.8% of vanadium, from 0.5% to 2.5% of tin.

3. Titanium base alloys consisting essentially of from 0.1% to 1.5% of lead, from 3% to 7% of aluminum, from 0.5% to 2.8% of vanadium, from 0.5% to 2.5% of 30 tin.

4. A titanium base alloy according to claim 1 consisting essentially of from 0.5% to 3.5% of zirconium.

5. A titanium base alloy according to claim 2 con-

sisting essentially of from 0.5% to 3.5% of zirconium.

6. A titanium base alloy according to claim 3 consisting essentially of from 0.5% to 3.5% of zirconium.

7. A titanium base alloy according to claim 1 which consists of up to 4% zirconium.

## References Cited in the file of this patent

## UNITED STATES PATENTS

|           |                     |               |
|-----------|---------------------|---------------|
| 2,669,513 | Jaffee et al. ----- | Feb. 16, 1954 |
| 2,669,514 | Finlay et al. ----- | Feb. 16, 1954 |
| 2,703,278 | Finlay et al. ----- | Mar. 1, 1955  |
| 2,754,204 | Jaffee et al. ----- | July 10, 1956 |
| 2,754,205 | Jaffee et al. ----- | July 10, 1956 |

## FOREIGN PATENTS

|           |              |               |
|-----------|--------------|---------------|
| 1,070,589 | France ----- | Feb. 29, 1954 |
| 1,085,628 | France ----- | July 28, 1954 |
| 1,094,705 | France ----- | Dec. 8, 1954  |